

Dec. 13, 1938.

J. G. FORD

2,139,945

HEAT TRANSFER FLUID

Filed March 15, 1935



WITNESSES:

C. J. Weller.  
H. J. Bryant

INVENTOR

James G. Ford.

BY

Frank J. Savage

ATTORNEY

## UNITED STATES PATENT OFFICE

2,139,945

## HEAT TRANSFER FLUID

James G. Ford, Forest Hills, Pa., assignor to  
Westinghouse Electric & Manufacturing Com-  
pany, East Pittsburgh, Pa., a corporation of  
Pennsylvania

Application March 15, 1935, Serial No. 11,259

21 Claims. (Cl. 252—1)

This invention pertains to heat transfer fluid of dielectric nature, useful for cooling or for insulating purposes, as in transformers and the like.

This case is a continuation-in-part of my application Serial No. 656,852, filed February 15, 1933, and assigned to the Westinghouse Electric & Manufacturing Company.

In network transformers, for example, such as are installed in congested city office buildings, hazards of public safety and of operating efficiency require the dielectric fluid to be explosion-proof. Consequently, it is desirable to eliminate oil and to substitute dielectrics that are non-flammable, but yet avoid introducing other deleterious qualities.

It is among the objects of this invention to provide generally useful heat transfer fluid, and more particularly suitable insulating and cooling fluid for electrical apparatus; to overcome defects of former insulating or cooling liquids, and to obtain a combination of suitable qualities, as subsequently to be described more fully. Particular objects comprise providing liquid of this sort that is non-flammable, that is relatively stable under electrical stress, and that will remain in liquid state over rather wide ranges of temperature. Other objects will appear from the following description and accompanying drawing of preferred embodiments of this invention.

I have discovered that certain combinations of halogenated compounds overcome many of the defects of such compounds and provide liquids that are feasible for use even in network transformers and the like.

This invention is predicated on my discovery that combinations involving certain halogenated compounds of the naphthalene series, certain halogenated compounds of the benzene series, and certain diphenyl compounds, in binary or even more complex combination with each other, exhibit qualities heretofore lacking in transformer liquid.

Reference is made to the accompanying illustrative drawing, showing conventionally a transformer comprising a tank 1, transformer elements designated as 2, and conductors 3. Protected within the tank is liquid 4 for cooling and insulating the transformer elements and leads.

For further illustration of the principles and present preferred practice of this invention, reference is made to specific embodiments thereof.

Suitable halogenated naphthalenes are dissolved in an appropriate base.

Trichlorobenzene has been suggested heretofore as a dielectric but for such uses it has proved to be unsatisfactory in various respects that have been difficult to overcome. This invention minimizes the undesirable properties of trichlorobenzene and utilizes certain of its valuable charac-

teristics to provide exceptionally useful composite dielectric liquid.

The trichlorobenzene known as the 1,2,4 isomer is selected, preferably, since it is a commercially available halogenated hydrocarbon that exhibits considerable solvent affinity for certain halogenated compounds, particularly for members of the naphthalene series of hydrocarbons which are to be utilized in the transformer liquid.

The symmetrical (1, 3, 5) isomer however is well adapted to the purposes of this invention. Other desirable qualities conducive to the value of the solvent dielectric in the mixture are relatively high chemical stability under electric stress; relatively low emulsification with water, so that simple dehydrating means may be used in the apparatus; relatively wide range of liquid state in the mixture, relatively low solvent or dispersing power for the cellulosic or resinous insulating varnishes used on the electrical conductors; stability against decomposition by oxygen, against the catalytic effect of moisture, of short wave or light radiation, or of incidental contaminating metals; relatively high resistance, low power loss and low ionizing power. It is not intended to limit this invention to pure 1,2,4, 25 trichlorobenzene though as the predominant base that liquid is preferred. Nor is this invention confined to trichlorobenzene base; for example, for some uses a portion or all of that compound may be replaced by other halogenated benzene, 30 such as by trifluorobenzene or by other halogenated hydrocarbons that have good solvent power, particularly for halogenated naphthalene.

Halogenated naphthalenes to be utilized according to this invention have of themselves been proposed as dielectrics, but not the more viscous higher or solid members thereof as insulating and cooling fluid for transformers, nor in relatively high concentration with solvent to form cooling liquid, nor combined with appreciable proportion of organic compounds, such as trichlorobenzene, which of themselves would possess many unsatisfactory characteristics for dielectric purposes, nor in solution with somewhat viscous halogenated hydrocarbon for producing low viscosity liquid.

The naphthalene element of this composite dielectric is illustrated by halogenated naphthalene mixtures such as chlorinated naphthalenes, often known as halowaxes. Though individual halogenated naphthalenes may be used, mixtures such as halowaxes offer various advantages. Though certain of these mixtures are liquid and may be used for the purposes of this invention, the preferred mixtures are of solid or waxy nature. Halowaxes ranging from about 54 percent chlorine to about 62 percent chlorine are illustrative, though not restrictive, of suitable species of this component. They yield combinations

with the solvent that exhibit suitably depressed freezing points for use at low-temperatures and suitably elevated vaporizing points for use at rather high temperatures. The particular species mentioned possess of themselves a melting point range of about 190°-280° F. and boiling point range of about 550°-700° F. These combinations of halowax and solvent further are relatively stable against electrical stress and against moisture, and also are of improved resistance to burning.

Though reference has been made to chlorinated naphthalene, this invention contemplates that other halogen derivative may be substituted therefor in whole or in part, and particularly fluorinated naphthalenes.

Further advantages of this invention are obtainable by modification of the solutions described. For example diphenyl ether is found to be soluble in these combinations. Even relatively small quantities impart increased solubility to the naphthalenes, and permit considerable decrease in proportion of the trichlorbenzene. Thus the liquid range of the dielectric is extended to lower temperatures, though high chemical stability and good electrical properties are retained. Quantities up to the order of ten or fifteen percent may be added for these purposes. Similarly diphenyl itself, or halogenated diphenyl, such as chlorinated or fluorinated diphenyl or chlorinated or fluorinated diphenyl oxide in small amount serve to improve the solubility of the naphthalenes and increase the availability of their desirable properties. In certain instances larger proportions of these halogenated compounds, for example, of the order of 50% by weight of the final mixture, may also be utilized with success in practicing my invention. In general the quantity of naphthalene dissolved may be increased with increase of the diphenyl component.

In providing dielectrics for network transformers, it is desirable to produce material which on electrical decompositions generates non-inflammable gases. This may be accomplished by following the teachings to be disclosed hereinafter.

The advantages of the present improved dielectric liquid may be enhanced further in accordance with a specific feature of this invention. The solutions herein disclosed possess the ability to dissolve fluorinated hydrocarbons of straight chain and of cyclic nature. Of such solutes in turn many possess the quality of eliminating not only fire point (sustained burning) but even of eliminating flash point from the composite dielectric. As an example of fluorinated straight chain hydrocarbon that is at present preferred because of its solubility, chemical and electrical resistance, and ability in very small quantities to eliminate fire hazard, reference is made to tetrachlorodifluoroethane,  $C_2Cl_4F_2$ . For example as little as one percent of this solute raises the flash point to 440° F. and minimizes the fire point until burning occurs only on superheating at the boiling point. The addition of three percent of this preferred fluorinated compound entirely eliminates both flash and fire points. Therefore three to five percent of this compound provides abundant excess for elimination of explosion or fire hazard from the dielectric.

To provide further against development of inferior dielectric qualities in this composite dielectric under adverse conditions of use, it may be desirable not only to remove moisture during use, as heretofore mentioned in this description, but also to minimize the development of hydroge-

nous decomposition products or of acid, or to remove any such products as may be formed. With avoidance of moisture accumulation, this composite dielectric is capable of extended contact with cellulosic insulations and the like without appreciable impairment of their structure or insulating qualities. For the purpose of avoiding development of such destructive influences in this dielectric, this invention comprises as a further, though optional, improvement treatment of the liquid by activated clay or fuller's earth, or other treating materials that will not contaminate the liquid, to remove any soluble electrically deleterious products, especially any of acidic nature.

A specific example of dielectric illustrative of one preferred embodiment of this invention is presented by

#### Formula I

Pounds 2

|                                                |      |
|------------------------------------------------|------|
| Halowax, halogenated naphthalene, about 54% Cl | 159  |
| Halowax, halogenated naphthalene, about 58% Cl | 159  |
| Halowax, halogenated naphthalene, about 62% Cl | 159  |
| Trichlorbenzene (predominantly 1,2,4 isomer)   | 677  |
| Diphenyl oxide                                 | 81   |
| Tetrachlorodifluoroethane                      | 25 3 |

These proportions may be varied, as for example, on a basis exclusive of the added fluorinated compound, from about twenty-five to sixty percent of the halowax components, about seventy to twenty-five percent of the solvent trichlorbenzene, and about five to fifteen percent of the diphenyl oxide, or similarly of equivalent components. In the above example the amount of tetrachlorodifluoroethane may vary from about twelve pounds to about sixty-five pounds, or from about one to five percent of the other elements of the solution. Tetrachlorethylene or penta-chlorethane to repress flash point may be desirable to the order of about fifteen percent.

The characteristics of this preferred embodiment of the invention comprise a specific gravity of 1.484 or about 1.5, and coefficient of expansion 0.00078° C.; no flash nor fire points and high resistance to deterioration by oxidation or by hydrolysis, solidification temperature at least 20° F., specific heat 0.40 calories/cubic centimeter, viscosity 34 seconds Saybolt at 100° F., or absolute viscosity 3 centipoises, power factor of well prepared solution 2 to 3 percent. Thus it is evident that in addition to substantially no fire hazard this solution is operative over a wide range of temperatures, and is well adapted as cooling liquid, because it possesses high specific heat and because its low viscosity and its rapid change of volume with temperature readily promote convection currents.

Further preferred embodiments of this invention utilize chlorinated diphenyl compounds in major proportions. The following specific example illustrates one such further embodiment.

#### Formula II

Pounds

|                                                                          |         |
|--------------------------------------------------------------------------|---------|
| Chlorinated naphthalene (about 50% to 62% chlorine)                      | 285.5 7 |
| Trichlorbenzene (predominantly 1,2,4 isomer)                             | 339.5   |
| Chlorinated diphenyl oxide or chlorinated diphenyl (about 50% to 68% Cl) | 643.0   |
| Diphenyl oxide                                                           | 45 7    |

As in the mixture of Formula I, the trichlorbenzene serves as a solvent for the other ingredients. The quantity of this trichlorbenzene, which when undiluted has a relatively high power factor, is kept as low as is consistent with proper solution of the other ingredients in order that the resulting final mixture may have a relatively low power factor.

The chlorinated naphthalene in the form of a solid wax is dissolved in the trichlorbenzene and serves to increase the halogen content of the final mixture. It also functions to raise the chemical stability of the liquid, reduces its viscosity, and lowers the over-all power factor.

15 The chlorinated diphenyl oxide (sometimes also designated as chlorinated phenyl ether) or the chlorinated diphenyl cooperates in dissolving the chlorinated naphthalene, thereby keeping down the content of trichlorbenzene. It is stable, tends 20 to improve the power factor of the final liquid, and by reducing the vapor pressure of the mixture prevents rapid losses by evaporation. In addition it furnishes additional available chlorine and retards crystallization of the chlorinated 25 naphthalene.

The diphenyl oxide serves, as in the mixture of Formula I, primarily to lower the freezing point. In addition, it acts as a solvent for the chlorinated naphthalene and thereby aids in keeping 30 down the total amount of trichlorbenzene.

This dielectric mixture is completely fireproof. The gases given off during decomposition are not combustible. In these gases hydrochloric acid fumes are present in a predominating proportion 35 and by their diluting effect minimize explosion danger due to any presence of free hydrogen.

The characteristics of this second embodiment of the invention comprise a specific gravity of 1.544 and coefficient of expansion of 0.00078 per 40 ° C. It has no flash or fire points and possesses high resistance to deterioration by oxidation or by hydrolysis. It has specific heat of 0.40 calories/cubic centimeter, a solidification temperature below -20° F., a viscosity of 58 seconds 45 Saybolt at 100° F., and a power factor of about one percent at 75° F. It possesses the same general advantages as does the first-named embodiment.

The above-stated proportions of Formula II 50 may, to obtain other given desired physical and electrical characteristics, be varied from about 15 to 30 percent for the chlorinated naphthalene component, about 15 to 60 percent for the chlorinated diphenyl oxide or chlorinated diphenyl 55 component, and about 15 to 45 percent for the trichlorbenzene component. The amount of diphenyl oxide may vary from 0 to about 10 percent of the other elements of the solution.

A third embodiment of my invention is presented by

### Formula III

Pounds

|                                                    |       |
|----------------------------------------------------|-------|
| Chlorinated naphthalene (about 54% Cl)             | 102.0 |
| Chlorinated naphthalene (about 58% Cl)             | 102.0 |
| Chlorinated naphthalene (about 62% Cl)             | 102.0 |
| Trichlorbenzene                                    | 404.2 |
| Chlorinated diphenyl oxide or chlorinated diphenyl | 510.0 |
| Diphenyl oxide                                     | 53.6  |

This mixture is basically similar to that of Formula II. The chlorinated naphthalene ingredients are comparable to those of Formula I in that they comprise a mixture of chlorinated 70 naphthalenes of differing chlorine contents. The

mixture has a specific gravity of 1.53 and a solidification temperature much below -20° F. It has no flash or fire points and possesses high resistance to deterioration. It has a specific heat and a coefficient of expansion substantially the same 5 as the solutions of Formulae I and II, a viscosity of 52 seconds Saybolt at 100° F., and a power factor also of about one percent.

The proportions of Formula III may be varied 10 to obtain other given desired physical and electrical characteristics throughout the same general ranges previously stated for Formula II.

For the purpose of further enhancing the fire-resistance characteristics of the mixtures of Formulae II and III, small quantities of a fluorinated straight chain hydrocarbon may be added thereto. Thus when the before-mentioned tetrachlorodifluoroethane is introduced in quantities up to 5% both flash and fire points are in all cases entirely eliminated from these chlorinated 20 diphenyl oxide and chlorinated diphenyl mixtures. When, however, the proportions are as stated by the two formulae last named, such additions are not ordinarily found necessary.

The fireproof compounds of this invention have 25 particular use in meeting high standards for dielectric such as are imposed for network transformers, but other uses now will be evident to those skilled in the art. For example, this dielectric is well suited for insulation of cables, such 30 as those commonly filled with oil. A cable of this type is represented conventionally by numeral 5 in the drawing, comprising this improved dielectric fluid 4. Liquid embodying the principles of this invention is particularly well suited as heat 35 transfer medium not only in strictly electrical apparatus but as cooling fluid for turbine bearings and the like, where severe requirements are imposed, particularly as to non-flammability or susceptibility to explosion.

According to the provisions of the patent statutes, I have explained the principle and mode of operation of my invention and have illustrated and described what I now consider to represent its best embodiments. However, I desire to have it 45 understood that within the scope of the appended claims, the invention may be practiced otherwise than as specifically illustrated and described.

I claim as my invention:

1. As a new composition of matter a fireproof 50 liquid at ordinary temperatures comprising at least fifteen percent of solid halogenated naphthalene compound in admixture with a liquid halogenated cyclic compound.

2. A dielectric liquid at ordinary temperatures 55 comprising an isometric mixture of trichlorbenzene, 1,2,4, trichlorbenzene predominating, and solid halogenated naphthalene compound in solution, said compound containing from fifty to seventy percent chlorine.

3. A liquid of dielectric nature at ordinary temperatures comprising in solution twenty-five to sixty percent solid halogenated naphthalene compound and trichlorbenzene.

4. A liquid of dielectric nature at ordinary temperatures comprising at least thirty percent of a mixture of chlorinated naphthalenes of aggregating from fifty to sixty-five percent chlorine in solution with trichlorbenzene.

5. A liquid of dielectric nature comprising in 70 solution halogenated naphthalene, trichlorbenzene and diphenyl compound, and fluorinated straight chain hydrocarbon for minimizing flash point.

6. A liquid of dielectric nature comprising in 75

- solution substantially thirty-five to forty percent chlorinated naphthalenes aggregating from fifty to sixty-five percent chlorine, from five to fifteen percent diphenyl compound, and the balance substantially trichlorbenzene, and in addition fluorinated straight chain hydrocarbon up to about fifteen percent to minimize flammability of the dielectric.
7. Liquid of dielectric nature comprising trichlorbenzene, halogenated naphthalene and fluorinated straight chain hydrocarbon for minimizing flash point.
8. Liquid of dielectric nature comprising trichlorbenzene, halogenated naphthalene and tetrachlorodifluoroethane for minimizing flash point.
9. A heat transfer system comprising liquid of trichlorbenzene and halogenated naphthalene base and up to the order of fifteen percent additional liquid to repress flash point selected from 20 a group consisting of fluorinated straight chain hydrocarbon, pentachlorethane and tetrachloroethylene.
10. A fireproof liquid of dielectric nature comprising in solution solid halogenated naphthalene, trichlorbenzene and diphenyl.
11. A fireproof dielectric liquid at ordinary temperatures comprising in solution solid chlorinated naphthalene, trichlorbenzene, and chlorinated diphenyl oxide.
12. A fireproof dielectric liquid at ordinary temperatures comprising in solution solid chlorinated naphthalene, trichlorbenzene and chlorinated diphenyl.
13. A fireproof dielectric liquid at ordinary temperatures comprising in solution solid chlorinated naphthalene, trichlorbenzene and diphenyl oxide.
14. A fireproof dielectric liquid at ordinary temperatures comprising in solution solid chlorinated naphthalene, trichlorbenzene, chlorinated diphenyl oxide, and diphenyl oxide.
15. A fireproof dielectric liquid at ordinary temperatures comprising in solution solid chlorinated naphthalene, trichlorbenzene, chlorinated diphenyl and diphenyl oxide.
16. As a new composition of matter, a fireproof liquid at ordinary temperatures comprising chlorinated naphthalene and solvent therefor in the form of trichlorbenzene.
17. As a new composition of matter, a fireproof liquid at ordinary temperatures comprising chlorinated naphthalene and solvent therefor in the form of trichlorbenzene and chlorinated diphenyl oxide.
18. As a new composition of matter, a fireproof liquid at ordinary temperatures comprising chlorinated naphthalene, halogenated solvent therefor, and a freezing point depresser in the form of diphenyl oxide.
19. A liquid composition adapted for electrical insulating and cooling purposes comprising substantial amounts respectively of solid chlorinated naphthalene and liquid chlorinated benzene, said composition having a materially lower pour point than either of said ingredients.
20. A liquid composition consisting substantially of chlorinated naphthalene, a halogenated phenyloid compound containing a plurality of phenyl groups and chlorinated benzene.
21. A liquid material suitable for use in electrical devices comprising essentially chlorinated naphthalene, a chlorinated diphenyl compound and trichlorbenzene.

JAMES G. FORD.